

July 28, 1936.

H. RUBEN ET AL

2,049,320

CIGARETTE

Filed Dec. 2, 1933

FIG. 1.



FIG. 2.



FIG. 3.



FIG. 4.



FIG. 5.



FIG. 6.



INVENTORS:

Hans Ruben,  
Moritz Salomonski,  
by Weichersborn,  
attorney.

## UNITED STATES PATENT OFFICE

2,049,320

## CIGARETTE

Hans Ruben, Berlin-Charlottenburg, and Moritz Salomonski, Berlin, Germany; said Ruben assignor to Elsbeth Ruben, Charlottenburg, near Berlin, Germany

Application December 2, 1933, Serial No. 700,710  
In Germany December 8, 1932

## 4 Claims. (Cl. 131—52)

Our invention relates to cigarettes, and it is an object of our invention to provide a cigarette with means for extinguishing its burning wrapper and tobacco filler, to prevent smouldering of discarded cigarettes.

To this end, we treat a zone of the wrapper with a compound which contains an impregnating agent of non-combustion supporting properties and an amorphous, organic and liquid-binding substance.

The non-combustion-supporting agent must not soak the wrapper, but penetrate only for a portion of its thickness so that the non-penetrated portion remains flexible and the paper does not become weak and brittle.

A suitable compound has the following composition, in per cent by weight:

|                                           |    |
|-------------------------------------------|----|
| Water glass ( $K_2SiO_3$ or $Na_2SiO_3$ ) | 49 |
| Glycerine                                 | 1  |
| Starch                                    | 25 |
| Talc                                      | 25 |

In this compound the waterglass is the non-combustion-supporting agent, and the starch is the amorphous, organic and liquid-binding substance. The glycerine and talc are added for imparting ductility and resiliency to the wrapper.

We are not limited to a compound of exactly the above composition but may vary the composition as required. In particular, the percentage of starch must be regulated in conformity with the water content of the water glass. Such regulation is by no means difficult. A desideratum is that the fourth part of the compound should be talc, and that 1% glycerine should be present. Therefore, the percentage of starch should be regulated so as to obtain a total percentage of 74 for the water glass and the starch.

Preferably, the amorphous compound is applied to the wrapper of the cigarette by spraying. As mentioned, the water glass impregnates the wrapper without soaking it, i. e., it penetrates only for a portion of the wrapper's thickness so that the balance of the wrapper remains flexible. By these means, only a superficial layer of the wrapper is penetrated by the impregnating liquid. The starch in the compound absorbs any excess of water which might soak the wrapper.

Any kind of starch may be used for the compound but preferably it should be fine grained and pure white so that the layer of amorphous compound is invisible on the wrapper.

As a rule, the compound is applied to the inner side of the wrapper, in the immediate vicinity of its tobacco filler, but it may also be applied to

the outer side of the wrapper, or both to the inner and outer sides thereof. Even in the last-mentioned case, with impregnated zones at both sides of the wrapper, the impregnating liquid does not soak the paper of the wrapper but leaves an intermediate zone of unimpregnated paper, as has been found by microscopic investigation.

The amorphous compound may be applied to the wrapper in a single operation and this is 10 obviously preferable with respect to the manufacture of the cigarettes but we may also subdivide the operation into two stages by first impregnating the wrapper, for instance, with water glass or alum, of such concentration that the 15 impregnating agent will not soak the wrapper, and thereupon applying the amorphous compound to the impregnated zone of the wrapper.

Any other substances may be admixed to the amorphous compound in addition to those recited above, but under all conditions the compound should contain glycerine and talc, preferably in the proportions of 1 and 25%, respectively, as otherwise the wrapper would not be as ductile and resilient as required.

A substance which is preferably admixed to the compound, is powdered metal or alloy, for instance, powdered bronze.

Our invention is performed with simple means and does not increase the cost of manufacture 30 while on the other hand cigarettes which have been treated according to our invention, are superior to those which are on the market at present.

The smouldering of discarded cigarette ends 35 is undesirable under all conditions, and often dangerous. Cigarettes smouldering in an ash tray are particularly unpleasant. Means for extinguishing discarded cigarette ends have already been proposed but they do not eliminate 40 the drawback altogether, apart from the fact that they require the smoker's attention.

It has been found that the smouldering of a cigarette is determined by the smouldering of its wrapper. The glowing portions of the wrapper 45 creep and ignite the tobacco of the filler but this ignition is secondary, provided, of course, that the cigarette has been discarded, i. e., the smoking has been discontinued. Smouldering is therefore prevented by extinguishing the flame in the 50 wrapper.

It has already been proposed, as described in U. S. patent to Weil, No. 1,555,320, September 29, 1925, for "Cigarette", to treat the paper of wrappers with a non-combustion supporting liquid but 55

the use of an amorphous compound is nowhere disclosed, nor does the patentee limit the penetration of the liquid into the wrapper.

The said patentee also proposes to provide a band on the cigarette for extinguishing its wrapper but this is not desirable as the band shows and renders the paper of the wrapper less ductile and flexible.

It has also been proposed to prevent smouldering by providing a layer on the wrapper, or by impregnating the wrapper.

A layer, in order to be effective, must be comparatively thick and it does not make a difference in this respect whether it is on the inner or on the outer side of the wrapper. Such a thick layer, however, renders the wrapper less flexible and this is particularly undesirable if the cigarettes are made mechanically.

Impregnation also involves certain difficulties. Firstly, an impregnation which is expected to be effective by itself, cannot be obtained in a fraction of a second which is the time available for the impregnation in modern cigarette manufacture. Secondly, an effective impregnation involves soaking of the wrapper throughout its thickness by which, as stated above, the flexibility and strength of the paper are reduced too much.

Our invention eliminates these drawbacks by associating the impregnated material with the layer. Preferably, in a cigarette having a layer of an amorphous and non-combustion supporting substance for preventing smouldering, the impregnation involves only the surface layer of the wrapper to which the said amorphous layer sticks. By these means, as described, a portion of the paper is unchanged and so the strength of the paper is not reduced to such an extent that the paper might break, and on account of the impregnation the amorphous layer can be comparatively thin.

A superficial impregnation of the wrapper in a cigarette, as described, and the subsequent coating with an amorphous and non-combustion supporting substance which may be metal powder, for instance, bronze powder, or may contain such powder, are effected without difficulty in up-to-date cigarette manufacture.

In the accompanying drawing, several adaptations of our invention are illustrated by way of example.

In the drawing

Fig. 1 is a perspective illustration of a cigarette with an impregnated zone at one end which extends through to the end of the cigarette.

Fig. 2 is an axial section, much enlarged, showing a portion of the wrapper of a cigarette in which the impregnated zone and the amorphous layer are on the inner, and

Fig. 3 is a similar section of a wrapper in which the zone and the layer are on the outer side of the wrapper.

Fig. 4 is a similar section in which one zone and one layer are on the inner, and another zone and another layer are on the outer side of the wrapper.

Fig. 5 shows a wrapper for the cigarette in Fig. 1, spread out, and

Fig. 6 shows a wrapper, also spread out, for a cigarette in which the impregnated zone is spaced apart from the adjacent end.

Referring now to the drawing, and first to Fig. 1, the cigarette comprises a wrapper 1, of any suitable material, and a tobacco filler 2 in the wrapper. An impregnated zone *i* extends in-

wardly on the wrapper 1 from the rear end of the cigarette.

As mentioned, the impregnated zone *i* is preferably on the inner side of the wrapper, as illustrated in Fig. 2. The compound containing the amorphous substance and an impregnating liquid may be applied to the inner side of the wrapper in a single operation, or the impregnating liquid may be applied first, and the amorphous compound is then applied to the impregnated portion of the wrapper. Under all conditions, however, the impregnating liquid, for instance, water glass or alum, should be of such concentration that it will not penetrate beyond a given depth, as indicated by the more closely shaded rectangle 3, and that a portion of the paper in the wrapper conserves its flexibility and strength, properties which are obviously deteriorated in the impregnated portion 3. 4 is the amorphous layer on the impregnated zone.

Fig. 3 shows the impregnated zone on the outer side of the wrapper 1. Otherwise, this section is quite similar to that in Fig. 2.

Referring to Fig. 4, the inner impregnated zone *i*, with the impregnated portion 3 and the layer 4 of amorphous substance, is combined with an outer impregnated zone *i*<sub>o</sub> which includes the impregnated portion 33 and the layer 44. It will appear that the paper of the wrapper 1 is not soaked throughout but has an unimpregnated section between the portions 3 and 33.

Fig. 5 shows the wrapper 1 for the cigarettes in Figs. 1 to 4, all of which have the impregnated zones *i* (or *i*<sub>o</sub> and *i*) extending as far as the rear end of the cigarette.

Fig. 6 shows a wrapper for a cigarette whose impregnated zone *I* is spaced apart from the rear end of the cigarette. This zone has been shown narrower than the zone *i* (or *i*<sub>o</sub> and *i*) only by way of example. Obviously it might be as wide as *i*, or *i* might be as narrow as *I*, as desired or required.

Our invention also relates to the method of applying the compound to the wrapper. This is effected by spraying the compound onto the wrapper. As compared with the usual method of pasting a band to the wrapper which may be said to be of a physico-chemical character, the spraying method is essentially mechanical and by regulating the spraying pressure the adhesion of the compound to the wrapper, and the depth to which the impregnating liquid penetrates into the wrapper, can be regulated.

We claim:

1. A cigarette comprising a wrapper, a tobacco filler, and a zone in said wrapper impregnated with a compound which contains water glass, glycerine, starch and talc.

2. A cigarette comprising a wrapper, a tobacco filler, and a zone in said wrapper impregnated with a compound which contains water glass, glycerine, starch and talc, the last-mentioned constituent making up one-fourth of the compound.

3. A cigarette comprising a wrapper, a tobacco filler, and a zone in said wrapper impregnated with a compound which contains water glass, glycerine, starch whose percentage is determined by the water content of the water glass, and talc.

4. A cigarette comprising a wrapper, a tobacco filler and a zone in said wrapper impregnated with a compound which contains 49% waterglass, 1% glycerine, 25% starch, and 25% talc.

HANS RUBEN.

MORITZ SALOMONSKI. 75